

F. A. FAHRENWALD,  
PROCESS OF COATING TUNGSTEN OR MOLYBDENUM ARTICLES WITH PRECIOUS METALS.  
APPLICATION FILED MAY 31, 1916.

1,261,110.

Patented Apr. 2, 1918.



Inventor  
Frank A. Fahrenwald.

By Hull, Smith, Brock & West

Attns.

# UNITED STATES PATENT OFFICE.

FRANK A. FAHRENWALD, OF CLEVELAND, OHIO, DEDICATED, BY MESNE ASSIGNMENTS, TO THE GOVERNMENT OF THE UNITED STATES OF AMERICA AND TO THE PEOPLE OF THE UNITED STATES OF AMERICA.

## PROCESS OF COATING TUNGSTEN OR MOLYBDENUM ARTICLES WITH PRECIOUS METALS.

1,261,110.

Specification of Letters Patent.

Patented Apr. 2, 1918.

Application filed May 31, 1916. Serial No. 100,997.

(DEDICATED TO THE PUBLIC.)

*To all whom it may concern:*

Be it known that I, FRANK A. FAHRENWALD, a citizen of the United States, residing at Cleveland, in the county of Cuyahoga and 5 State of Ohio, have invented a certain new and useful Improvement in Processes of Coating Tungsten or Molybdenum Articles with Precious Metals, of which the following is a full, clear, and exact description, 10 reference being had to the accompanying drawings.

This application is made under the act of March 3, 1883, chapter 143 (22 Stat., 625) and the invention herein described and 15 claimed may be used by the Government of the United States or its officers or employees in the prosecution of work for the Government or any person in the United States without the payment of any royalty thereon.

20 This invention relates to a metal body consisting of tungsten, molybdenum, or other oxidizable metal, and a layer of precious or non-oxidizable metal intimately connected therewith so as to permit the soldering, or brazing of the article, or other high temperature working thereof without the occurrence of oxidation.

Tungsten, particularly in the malleable and ductile states described in the patent of 30 William D. Coolidge, No. 1,082,933, dated December 30, 1913, is a most extraordinary metal by reason of its rigidity, hardness, tensile strength, insolubility, high melting point and other physical and chemical properties. Furthermore it has this peculiarity, 35 that any desired manipulation may be performed upon it whatsoever without drawing its temper or changing its state, provided the temperature to which it is subjected be 40 maintained lower than the critical point of its creation, which my experiments indicate to be somewhere between 1400 and 1500° C. The same properties are present in even higher degree in the alloy of tungsten and 45 molybdenum described in my application

filed June 3, 1916, Serial No. 101,502. However a disadvantage has been that it oxidizes very easily upon its surface at any temperatures higher than a dull red (say 600° C.) and, owing to this property and to the small 50 affinity which it possesses for different soldering elements, it was for a long time found impossible to weld, solder, braze, or otherwise unite different parts of these metals. These two drawbacks, of easy oxidation and 55 difficult soldering, have constituted the only impediments to the extensive use of these metals in dentistry and in many other practical arts, as well as in numberless scientific and philosophic uses.

60 The first solution attempted lay in searching for alloys which would preserve the beneficial properties of the material while avoiding its harmful properties, and to this end various attempts were made to secure an 65 alloy of tungsten in connection with gold, platinum, palladium and the like noble metals, but in most cases the affinity of tungsten for such other metals is so small and the difference between their melting points 70 so great that no alloy could be secured. However it was discovered that while the large pieces of tungsten were not appreciably dissolved they were nevertheless removed from the molten bath with a beautiful 75 impervious coating. As either of these furnished the surface qualities which tungsten lacks the two remaining conditions seemed to be fulfilled. And so they were; but after this bath the tungsten wires were 80 as brittle as glass. The problem thus arose of applying a coating of such material and under such conditions that the other valuable properties of the tungsten would not be destroyed during the process. The crystallization 85 of the tungsten was obviously due to one of three, or a combination of three causes: improper coating temperature, improper composition of the coating material, or improper time element.

90

A short resumé of my results is given in the following table, since it was discovered that only the metals silver, gold and palladium offered promise of complete success.

*Experiments in coating tungsten with gold, silver, and palladium, under varying conditions.*

| Composition. |           |           | Time.    | Temperature of bath. |                |                     |                |                       |                   |                     |                   |       |
|--------------|-----------|-----------|----------|----------------------|----------------|---------------------|----------------|-----------------------|-------------------|---------------------|-------------------|-------|
|              |           |           |          | 1,100° C.            |                | 1,350° C.           |                | 1,500° C.             |                   | 1,600° C.           |                   |       |
| Ag.          | Au.       | Pd.       |          | Effect on tungsten.  | Coating.       | Effect on tungsten. | Coating.       | Effect on tungsten.   | Coating.          | Effect on tungsten. | Coating.          |       |
| Per cent.    | Per cent. | Per cent. | Seconds. | 10                   | None.....      | Very poor.....      | None.....      | Very poor.....        | Very brittle..... | Poor.....           | Very brittle..... | Poor. |
| 100          | 100       | 100       | 30       | None.....            | Very poor..... | Quite brittle.....  | Very poor..... | Very brittle.....     | Poor.....         | Very brittle.....   | Poor.             |       |
|              |           | 100       | 10       | None.....            | Good.....      | None.....           | Good.....      | Slightly brittle..... | Good.....         | Very brittle.....   | Good.             |       |
|              |           | 100       | 30       | None.....            | Good.....      | None.....           | Good.....      | Quite brittle.....    | Good.....         | Very brittle.....   | Good.             |       |
|              |           | 100       | 10       |                      |                |                     |                | Quite brittle.....    | Good.....         | Very brittle.....   | Good.             |       |
|              |           | 25        | 10       |                      |                |                     |                | Very brittle.....     | Good.....         | Very brittle.....   | Good.             |       |
|              |           | 50        | 10       |                      |                |                     |                | Very brittle.....     | Good.....         | Very brittle.....   | Good.             |       |
|              |           | 75        | 25       |                      |                |                     |                | Very brittle.....     | Good.....         | Very brittle.....   | Good.             |       |
|              |           | 90        | 10       |                      |                |                     |                | Very brittle.....     | Good.....         | Very brittle.....   | Good.             |       |
|              |           | 95        | 5        |                      |                |                     |                | None.....             | Good.....         | Very brittle.....   | Good.....         |       |
|              |           |           | 10       |                      |                |                     |                | None.....             | Good.....         | Very brittle.....   | Good.....         |       |

These tests were made on drawn wires of 30-mil size, which without the coating, and heated in an atmosphere of hydrogen, crystallized and became brittle at 1,700° C. in from 10 to 20 min.

5 Silver alone may be employed but adheres rather weakly and appears for some unknown reason to accelerate crystallization in the tungsten, wherefore its use alone is not recommended. Platinum alone, and 10 certain other metals such as iridium, have a marked dissolving effect, and some of them therefore adhere very tenaciously to the surface of the tungsten. However platinum requires very delicate manipulation 15 since its melting temperature is dangerously close to the equiaxing temperature of the tungsten. Palladium alone adheres very strongly to and even alloys slightly with the tungsten, but also, when used alone, 20 appears to accelerate crystallization, though when used in company with a preponderance of gold this deteriorating effect is not observable. Gold alone has comparatively little affinity for tungsten, and the line of 25 contact is rather clearly defined, though it adheres reasonably well for all practical purposes and forms a most suitable coating without any injury to the metal beneath; but by adding small amounts of palladium 30 to the coating bath its melting point is raised, and, at the same time, a better bond between the tungsten and this protective layer is obtained. It will be noted from the foregoing table, that with a preponderance 35 of palladium in the coating bath the tungsten came out very brittle, but that when the palladium content was reduced to five or ten per cent. the bath could be reduced in temperature to 1350° C., and no effect was 40 produced upon the tungsten within the length of time necessary for the coating operation.

The time and temperature constants appear to be interdependent, the ductile tungsten undergoing a crystalline rearrangement 45

either upon a short exposure to a high temperature or a longer exposure to a lower temperature. Thus I have found that a subjection of the ductile tungsten to a temperature of 1400° C. or even 1450° for five or ten seconds will ordinarily not injure the metal, though I consider ten seconds at 1400° C. or thirty seconds at 1350° C. the maximum that should be considered for practical shop or technical uses.

I have discovered that this coating process may be performed in the open atmosphere by the use of a suitable flux. In small quantities the tungsten articles may be dipped into a bath of fused sodium carbonate, 60 sodium borate, or other oxygen alkali salt which will combine with the superficial oxides of the tungsten to form a suitable tungstate which is soluble in the bath. The tungsten article can then be removed from 65 this bath with a cleansing and protective shell of flux adhering to it, and dropped into the metal bath whereupon the flux is automatically removed and the metal coating acquired. For the larger scale treatment of 70 tungsten wire I have supported the wire in such a way that a bight or downwardly extending loop of the wire should dip beneath the surface of fused alkali in a flaring receptacle and passed through a molten button of coating metal located at the bottom thereof. The tungsten wire being drawn uniformly through this bath, the coating operation become continuous, the portions 75 of the wire outside the bath being, of course, maintained sufficiently cool to prevent oxidizing.

Either of these processes results in a wire or article having a coating of gold or other precious metal thereon of considerable 85 thickness, owing to the adhesion of the gold.

However if the time and temperature elements above mentioned are kept within the limits indicated, the strength, rigidity, ductility and tensile strength of the tungsten 5 will not be in any way impaired, but the metal becomes proof against oxidation and can be soldered with the greatest ease, wherefore the resulting article will be found suited for uses which have heretofore been 10 satisfied only by such expensive materials as platinum and platinum iridium alloys.

In the drawings accompanying and forming a part of this application I have illustrated various manipulations for effecting 15 this coating operation, some of the same being confined to use with wire, and others being susceptible equally for the coating of other shapes or articles. In these drawings Figure 1 represents the simplest operation, 20 merely of dipping in an open crucible under the surface of a flux; Fig. 2 represents the drawing of a wire through a perforated crucible; Fig. 3 represents the drawing of a wire through a button of melted gold 25 under flux; and Fig. 4 represents a dipping operation performed in a reducing or inert atmosphere.

In Fig. 1, 1 represents a crucible of any suitable type, 2 a blast lamp or other heating element, 3 a button of the molten metal which may be gold or an alloy of gold or other noble metal or alloy as above described; and 30 4 represents the flux. 5 represents the article to be coated, here shown as a dental pin 35 held in suitable tongs 6, the tongs preferably having porcelain or the like grasping points in order that the distribution of the gold upon the article may not be affected thereby. With the ordinary Bunsen burner or with 40 the ordinary blast lamp, unless very powerfully urged, there is no danger of obtaining a temperature so high as to equiaxiate the tungsten. It is obvious that disks, cylinders or other shapes could equally well be 45 coated as the wire or rod shown.

In Fig. 2 I have illustrated an arrangement whereby a wire can be coated by a continuous operation. In this view the crucible 10 is illustrated as formed with an aperture 50 11 in its lower part closely receiving the wire 12. The mass 13 of the desired coating metal is fused within the crucible in any suitable manner, preferably beneath the surface of a flux 14, although in this case I do not consider 55 the flux indispensable. The wire 12 being drawn steadily upwardly at the requisite speed, which can be easily ascertained by observation for a few seconds, a perfect coating of metal will be deposited thereon. 60 By suitably arranging the heating appliance (not shown) and by mechanically scraping or cleaning the wire before drawing the same into the metal, the coating will adhere

sufficiently without other precautions. The coating of metal upon the wire after it emerges above the molten metal will sufficiently prevent any oxidation or other change in the same, although a flux of some nature is frequently desirable to increase the fluidity of the metal and to restrain its 70 cooling.

In Fig. 3 I have illustrated another expedient for the continuous coating of a wire. In this view I have illustrated an electrical resistance furnace comprising a carbon rod 20, suitably hollowed cut or recessed at 21 and traversed by a porcelain or other suitable stud 22. Suitable metallic terminals 23-23 are clamped against the ends of the carbon rod and provided with electrical 75 energy by the cables 24-24. The heat produced in the carbon melts the gold or other coating metal illustrated at 25, and also the flux 26 overlying the same, so that a wire 27 introduced beneath the stud 22 and pulled 80 in either direction will become cleansed and 85 coated in a single operation.

In Fig. 4 I have illustrated an electrical resistance furnace comprising resistance wires 30 coiled about the exterior of a tube 90 31, said tube having at one end the closure 32 connected with the pipe 33 through which some inert gas like nitrogen or some reducing gas like hydrogen can be forced. The gold or other coating metal is shown at 34 95 contained in a boat 35 and the article 36 to be coated is handled by means of the tongs 37, a suitable shield 38 being employed if desired. It will be understood that the above are only a very few of the arrangements and manipulations which could be 100 employed to the end in view.

While I have described my improved process chiefly in connection with tungsten, it is to be understood that the word molybdenum could be substituted in this specification wherever the word tungsten has been used, since the properties of the two metals are very similar, and I likewise consider the alloy of tungsten and molybdenum as comprised within the meaning of this specification equally with the metallic tungsten. 110

Having thus described my invention, what I claim is:

1. In the process of soldering oxidizable 115 metals like tungsten or molybdenum or their alloys, the step which consists in first coating said oxidizable metal with a non-oxidizable metal as gold, silver, platinum, palladium or an alloy thereof.

2. The process of coating tungsten and molybdenum with a precious metal, as gold, which consists in applying the coating metal in molten form in connection with a flux containing the oxygen salt of an alkali metal. 120

3. The process of preparing articles of

ductile tungsten and molybdenum for soldering or brazing which consists in heating such articles for not longer than about 30 seconds to a temperature of not more than 5 about 1350° C. in contact with molten gold and a flux containing the oxygen salt of an alkali metal.

4. The process of coating ductile tungsten with gold which consists in first immersing 10 said tungsten in a bath containing the fused oxygen salt of an alkali metal, and, second, immersing said article for not more than about 30 seconds in a bath containing principally or entirely molten gold at a temperature 15 of not more than about 1350° C.

5. The process of coating tungsten or molybdenum wires with a non-oxidizable metallic coating such as gold, silver, plati-

num or palladium, which consists in drawing said wires first through a bath containing the molten oxygen salt of an alkali metal and thereafter through a bath of the molten coating metal maintained at a temperature not higher than about 1400° C. 20

6. The process of treating tungsten or 25 molybdenum, comprising using as a flux a mixture consisting of or containing the oxygen salt of an alkali metal substantially as specified.

7. The process of treating tungsten or 30 molybdenum, consisting in coating it with a compound containing gold and palladium.

In testimony whereof, I hereunto affix my signature.

FRANK A. FAHRENWALD.